

M. Y. SEATON & J. S. HARRIS.  
PLASTERED CONCRETE CEILING AND METHOD OF MAKING SAME.  
APPLICATION FILED MAR. 23, 1917.

1,300,493.

Patented Apr. 15, 1919.



INVENTORS  
Max Y. Seaton  
and  
John S. Harris -  
BY Fay, Oberlin & Fay  
ATTORNEYS

# UNITED STATES PATENT OFFICE.

MAX Y. SEATON AND JOHN S. HARRIS, OF CLEVELAND, OHIO, ASSIGNORS TO THE ABCO COMPANY, OF CLEVELAND, OHIO, A CORPORATION OF OHIO.

## PLASTERED CONCRETE CEILING AND METHOD OF MAKING SAME.

1,300,493.

Specification of Letters Patent.

Patented Apr. 15, 1919.

Application filed March 23, 1917. Serial No. 156,898.

To all whom it may concern:

Be it known that we, MAX Y. SEATON and JOHN S. HARRIS, citizens of the United States, and residents of Cleveland, county 5 of Cuyahoga, State of Ohio, have jointly invented a new and useful Improvement in Plastered Concrete Ceilings and Methods of Making Same, of which the following is a specification, the principle of the invention 10 being herein explained and the best mode in which we have contemplated applying that principle, so as to distinguish it from other inventions.

The present invention, relating as indicated to a plastered concrete ceiling and method of making same, has more particular regard to the application of a plaster coat to a concrete surface by the use of an intermediate binder of a cementitious substance, which will produce a composite structure of considerable strength, and one which will not fail even under the most adverse conditions. To the accomplishment of the foregoing and related ends, said invention, then, consists of the means hereinafter fully described and particularly pointed out in the claims.

The annexed drawing and the following description set forth in detail one method 30 and one product exemplifying our invention, such disclosed procedure and product constituting however, but one of various applications of the principles of our invention.

In said annexed drawing:—

35 The single figure there appearing is a cross-sectional view illustrating a ceiling constructed in accordance with the principles of our invention.

Considerable difficulty has been found in 40 the application of plaster to concrete surfaces, and in particular to the application of plaster to concrete ceilings where the weight of the plaster must be held by the bond between the plaster and the concrete.

45 It is customary to first apply a thin coating of a heavy bituminous paint to the concrete surface and to then apply the plaster coats against this painted surface, but this method is unsatisfactory, and is not permanent, the 50 plaster often falling off after only a very few years of use. The bonding efficiency of such a paint is low however and its chief advantage is obviating the wetting down of the walls which must be done if plaster is ap-

plied direct. In some cases sand is blown 55 against and into this paint to roughen its surface and increase its effectiveness as a bond but even this step does not render the material satisfactory. The only method that has been found to be entirely satisfactory is to attach metal lath to the concrete ceiling and to then apply the plaster against this lath, but this method involves a very considerable expense and is not largely used for this reason. 60 65

The present invention involves the use on the concrete surface of a bonding substance, against which the plaster may be applied. The substance which we prefer to use is a drying oil which has been treated in a varnish kettle to render it viscous, and in which there is mixed a considerable quantity of fibrous material, such as asbestos or a silicate to increase its body. Various oils 70 may be used, such as china-wood oil, linseed 75 oil, soy-bean oil, or in fact any good drying oil. These oils are first treated by methods known to varnish makers to increase their viscosity and a large amount of short asbestos fiber is then mixed with the oil to 80 increase its strength. It is essential that this substance be inert in the presence of alkalis and insoluble in water since both alkalis and water are found to some extent in the concrete against which this substance is applied and in the plaster which is subsequently applied to the partially dried substance. The oil when treated may of course 85 be thinned with suitable agents such as turpentine or turpentine substitute until it is 90 sufficiently plastic for working and spreading.

The preferred method of the application of this substance to a concrete surface is by 95 troweling the same over the surface to a thickness of from between one sixteenth and one thirty-second of an inch, which is about the least thickness which a mason can conveniently apply the material by means of a trowel. At this thickness 25 pounds of 100 the material will cover about 100 square feet of surface, although we have found that good results can still be obtained by the application of the substance in various amounts. 105

After the viscous oil has been applied to the concrete the first plaster coat is applied before the bonding substance is thoroughly

2  
dry, which, under ordinary conditions, will be between one-half hour and three hours, and the best results are obtained by applying the plaster within one hour after the oil 5 has been applied. One, two or even more coats of plaster may be applied, as is customary in plastering practice under different conditions and the bond between the plaster and the concrete will of course depend upon the strength of the union, between the first plaster coat, the intermediate 10 cementitious or bonding substance and the concrete.

The strength of the ceiling formed in accordance with our invention depends to some 15 extent upon the composition of the plaster, but even with the weakest form of plaster ordinarily used, which is a white finish consisting of four parts of lime to one part of plaster of Paris, an excellent bond is obtained between the plaster and concrete and a ceiling of satisfactory strength is obtained.

Referring to the figure in the drawing, there is shown a concrete ceiling 1 upon 25 which has been applied a coating of our bonding substance 2. Upon the latter is the first or scratch coat of plaster 3 and on this plaster the final coat 4. Obviously the number of plaster coats may be varied to suit 30 the conditions and finish required. A brown coat (the coat 3) is ordinarily used where the surface of the concrete is so rough, due to form marks, air pockets and projecting lumps of aggregate that the bonding coat 35 does not serve to give a smooth surface. In case a brown coat is necessary we have found that very satisfactory results are obtained by using a mixture of four or five parts of sand to one part of hard wall plaster, or 40 gypsum plaster, preferably also with the addition of hair. This mixture is then, of course, brought to a workable condition by the addition of a suitable amount of water. In the brown coat lime may be substituted 45 for a part of the hard wall plaster, but as the use of lime diminishes the strength of the plaster, only a small amount should be used, as it is desirable that this coat have considerable structural strength.

50 If the concrete has a sufficiently smooth surface so that when the bonding substance is applied thereover a relatively smooth and uniform surface is secured, a white or finished coat of plaster may be applied directly 55 to the cementitious substance. We have found that a white finish of a standard composition comprised of four parts of lime to one part of plaster Paris gives very good results when thus applied directly, but such 60 a finish is rather weak, and in order to prevent dusting of this finished coating it is sometimes advisable to strengthen it by the use of a small amount of hard wall plaster. A composition which we have found very

satisfactory for this coat consists of four 65 parts of lime, one part of plaster of Paris and from one-half to one part of hard wall plaster.

If a sand finishing coat is applied a cementitious substance of a somewhat harder 70 material should be used than is commonly found under this name. A very satisfactory composition consists of four parts of sand, one part of lime, three-fourths to one part of neat wall finish and one-half to one part 75 of plaster Paris. If desired the lime can be replaced directly with neat wall finish and the setting time can be suitably regulated by the addition of plaster of Paris.

In all cases the plaster may be applied 80 according to standard plastering methods without the use of more force in applying the plaster than is commonly used in applying such material directly against lath or against the concrete surface. The white and 85 sand finishes can be worked to as thin a coat as is possible both for economy and efficiency.

It has been found by thorough tests that a ceiling of this type will resist excessive vibration and heat without any loss of strength 90 and without any falling of the plaster such as occurs under ordinary methods whenever a ceiling is subjected to any amount of vibration or any unusual temperature. Furthermore the bond is not affected by oxidation 95 since it is practically completely protected by the concrete on one side and the plaster on the other, and in the tests which have been made oxidation has never been found to be a source of failure. Test made 100 to determine the absorption of the oil by the concrete also shows no great deterioration and no failures from this condition. On the other hand efflorescence of various salts on 105 the surface of the concrete prevents the obtaining of a good bond between our improved substance and the concrete, and the substance should never be applied until the efflorescence has been entirely removed from the concrete, if a permanent ceiling is desired. The cost of a ceiling constructed in 110 accordance with our invention is practically the same as one made by the application of plaster to a bituminous paint applied to the concrete and is less than one-half the cost 115 of a suspended ceiling, that is, one made by applying the plaster to metal lath laid over the concrete.

Other forms may be employed embodying 120 the features of our invention instead of the one herein explained, change being made in the form of construction, provided the elements stated by any of the following claims or the equivalent of such stated elements be employed, whether produced by our preferred method or by others embodying steps 125 equivalent to those stated in the following claims.

We therefore particularly point out and distinctly claim as our invention:—

1. In a method of applying plaster to a concrete surface, the steps which consist in 5 first coating a set concrete surface with a viscous drying oil or varnish capable of drying at a speed greater than its absorption by the subsequently applied plaster to a thickness permitting the forcing thereinto of 10 the sand of a plaster coat, and then applying such plaster coat before the oil has thoroughly dried.

2. In a method of applying plaster to a concrete surface, the steps which consist in 15 first coating a set concrete surface with a viscous drying oil or varnish capable of drying at a speed greater than its absorption by the subsequently applied plaster to a thickness permitting the forcing thereinto of the 20 sand of a plaster coat, and then applying such plaster coat before the oil has thor-

oughly dried and forcing the sand of such plaster coat into such oil.

3. A composite wall structure consisting of a set concrete layer, a plaster layer, and 25 an intermediate layer cementing together such concrete and plaster layers, said intermediate layer consisting of a viscous drying oil containing fibrous material.

4. A composite wall structure consisting 30 of a set concrete layer, a plaster layer, and an intermediate layer of relatively slight thickness cementing together such concrete and plaster layers, said intermediate layer consisting of a binder containing a viscous 35 drying oil capable of drying at a speed greater than the absorption by the plaster and the concrete layers of the oil.

Signed by us, this 13 day of March, 1917.

MAX Y. SEATON.  
JOHN S. HARRIS.